# EUROPEAN PATENT SPECIFICATION

(11) **EP 0 815 985 B1**
(45) Date of publication and mention of the grant of the patent: **05.09.2001**
(21) Application number: 97109605.2
(22) Date of filing: 12.06.1997
(51) Int. Cl.: B21K 21/16, B21D 26/02, B21C 23/14

(54) **Method and apparatus for the hot-forming of tubular box-type elements of any shape made from a light alloy**
Verfahren und Vorrichtung zur Warmumformung von kastenförmigen Hohlprofilen irgendeiner Form aus Leichtmetall
Procédé et dispositif pour le formage à chaud d'éléments tubulaires en forme de caisson de forme quelconque en alliage léger

(30) Priority: 21.06.1996 IT TO960536
(43) Date of publication of application: 07.01.1998
(73) Proprietor: FIAT AUTO S.p.A., 10135 Torino (IT)
(72) Inventor: Da Re', Mario, 10100 Torino (IT)
(74) Representative: Plebani, Rinaldo

(56) References cited:
- EP-A- 0 294 034
- EP-A- 0 727 343
- PATENT ABSTRACTS OF JAPAN vol. 010, no. 207 (M-500), 19 July 1986 & JP 61 049735 A (RYODA SATO), 11 March 1986,
- PATENT ABSTRACTS OF JAPAN vol. 013, no. 013 (M-783), 12 January 1989 & JP 63 224857 A (KAWASAKI HEAVY IND LTD), 19 September 1988,
- PATENT ABSTRACTS OF JAPAN vol. 017, no. 043 (M-1360), 27 January 1993 & JP 04 262819 A (SHOWA ALUM CORP), 18 September 1992,
- PATENT ABSTRACTS OF JAPAN vol. 95, no. 002 & JP 07 032076 A (MITSUBISHI ALUM CO LTD;OTHERS: 02), 3 February 1995,

## Description

The invention relates to a method according to the preamble of claim 1 (see e.g. JP-A-07 032 076) of carrying out the hot-forming of tubular box-type elements (simply called "boxes" below) made of a light alloy (based on aluminium and/or magnesium for example) having the most diverse and complex shapes, both in transverse section and in the longitudinal direction. Box-type elements of this kind are used in particular in the motor industry as structural elements of the body of vehicles. The invention also relates to an apparatus suitable for implementing the method according to the invention.

It is known to produce some box-type structural elements of the body of vehicles by means of extrusions formed from light alloy; the known elements can, however, be formed only with relatively simple shapes, both in transverse section and, above all, in the longitudinal direction; in fact, the extrusion operation enables blanks to be obtained which generally have only a rectilinear shape; to obtain curvilinear elements, therefore, the extrusions subsequently have to be bent, with expensive additional working operations and the risk of breaking them because of the hollow internal structure.

To date, therefore, box-type elements of complex shape have been obtained in sheet steel or another material which is easy to weld (in contrast to aluminium and light alloys in general) and produced precisely by longitudinal welding of several profiles of open transverse section. In this way, however, the boxes have high weights, which mean higher costs, greater fuel consumption and increased pollution.

It is also known from JP 07 032076 a method according to which, after an extrusion phase, the extruded tube is moulded in the desired shape: the moulding phase is difficult to be performed and the method does not allow a high degree of accuracy of the tubular box to be achieved.

The object of the invention is to overcome the disadvantages described, by providing a method that is relatively simple, inexpensive and which does not require complex or cumbersome pieces of equipment, to form box-type elements made of any light alloy available on the market in any form or shape, with a high degree of accuracy and the minimum of waste.

On the basis of the invention a method is therefore provided for the hot-forming of a tubular box of any shape made from a light alloy, comprising a first phase in which the alloy is hot-extruded through a die of suitable shape so as to be formed into a tube of pre-determined section and generally rectilinear, and a moulding phase, in which the extrusion is pressed, to obtain the box of desired shape, between at least two moulds provided with respective conjugated cavities capable of defining with their contour the final shape of the box; characterized in that during the said moulding phase, the said moulds are kept close to each other in a fluid-tight manner; the said moulds being heated so as to maintain the extrusion, during the entire moulding phase, substantially at the same temperature at which it left the first extrusion phase; the moulding phase being carried out by creating a vacuum between extrusion and cavities, inside the cavities, and conveying a pressurized gas inside the extrusion.

Furthermore, the method of the invention preferably also comprises a second phase in which the extruded tube, still hot, is fed between the said moulds provided with conjugated cavities, during this second phase the moulds being heated so as to maintain the extrusion substantially at the same temperature at which it left the first extrusion phase; during the second phase the moulds being kept close together at a certain distance apart from each other, so that the cavities define a guide channel for the extrusion, inside which the latter is caused to slide so as to obtain a pre-form of it. It is understood that the above-mentioned phases are carried out sequentially and in the shortest possible time.

In this way, an extrusion that is substantially rectilinear and of simple shape in transverse section may be pre-formed in the longitudinal direction into any desired shape (U, L, zigzag, etc., for example), obtaining the hot bending thereof without the risk of breaking the transverse section and without having to resort to suitable bending equipment, and can then be moulded into a shape of transverse section of any complex design (H, star, etc.), still without any risk of breaking its transverse section.

The invention also relates to an apparatus for the hot-forming of a tubular box of any shape made from a light alloy, comprising an extrusion station capable of providing a tubular extrusion of pre-determined section and generally rectilinear, and a moulding station comprising at least two moulds provided with respective conjugated cavities capable of defining with their contour the final shape of the box to be obtained; characterized in that the said moulding station is arranged immediately downstream of the extrusion station, to receive said extrusion leaving the extrusion station directly between said moulds; the said moulds being provided with heating means and the moulding station also comprising:
- means for keeping the moulds selectively arranged in two different operating positions, in a first of which the moulds are close together at a certain distance apart from each other, so that the cavities define a guide channel for the extrusion provided with a through open end facing the extrusion station and through which the extrusion is capable of sliding in the channel so as to be pre-formed by it; and in a second of which the said moulds are kept close together in a fluid-tight manner; and
- means which can be actuated in the said second operating position of the moulds to create a vacuum between extrusion and cavities, inside the cavities, and to convey a pressurized gas inside the extrusion.

This and other features of the invention will be described in greater detail in the description which follows of a preferred embodiment which is given by way of non-exhaustive example with reference to the accompanying drawings, in which:
- Fig. 1 shows a diagrammatic view of the apparatus of the invention during the performance of some phases of the method according to the invention;
- Fig. 2 shows a detail of Fig. 1 on an enlarged scale and, diagrammatically, a further phase of the method of the invention, and
- Fig. 3 shows an exemplary transverse section of box obtainable according to the invention, compared with the overall dimensions of an extrusion from which it can be obtained, illustrated in dashed lines together with the profile of the cavities of two moulds brought close together for the pre-forming of the extrusion.

With reference to Figs. 1 to 3, in its entirety 1 shows an apparatus which can be used according to the invention to obtain the hot-forming of a tubular box 2 of any shape (in the non-exhaustive example shown the box 2 is U-shaped in longitudinal direction and rectangular transverse section) made of any light alloy.

The apparatus 1 comprises an extrusion station 3, of known type, capable of carrying out a first phase, that of extrusion, of the method of the invention to provide a tubular extrusion 4 of pre-determined section (circular in the non-exhaustive case shown) and generally rectilinear, and a moulding station 5 (capable, as will be seen, of carrying out a second and a third phase of the method of the invention) comprising at least two moulds 6, 7 (of which 7, the top one, is shown in Fig. 1 in a phantom view, so that the bottom mould 6 can be seen) provided with respective conjugated cavities 8, 9 (see also Fig. 3) capable of defining with their contour the final shape of the box 2 to be obtained (in this case the cavities 8, 9 are configured in a U on plan and have a rectangular transverse section).

According to the invention, the moulding station 5 is arranged immediately downstream of the extrusion station 3, to receive the extrusion 4 leaving the extrusion station 3 directly between the moulds 6, 7, so that when the extrusion begins to be worked in the station 5 it is still substantially at the same temperature at which it left the station 3; for this purpose, for example, the two stations 3 and 5 are arranged adjacent to one another and are connected by conveying means, such as a motor-driven roller conveyor 10, which is known, and which is capable of taking the extrusion 4 when it leaves the station 3 and causing it to advance, with pre-determined force, towards and inside the station 5. It is clear, therefore, that the stations 3 and 5 could also be adjacent or contiguous, and in this case the conveying means, particularly the roller conveyor 10, would be of dimensions which are reduced or actually absent, the feed force being conveyed to the extrusion directly by the action of the extruder.

The station 3 is preferably of the type that is capable of being fed with billets 11 of pre-determined dimensions and weight, obtained directly from the molten light alloy; these billets 11 are obtainable on the market and are fed to the station 3 in known manner, by means of handling devices 12, after having been pre-heated in a furnace to a pre-determined temperature which is suitable for rendering plastic (under suitable pressure) the alloy from which they are formed; in particular the station 3 includes an extrusion press 13, which is known, and illustrated solely in diagrammatic form, into which the red-hot billets (as is illustrated pictorially in Fig. 1) are introduced one at a time, and a matrix (or die) 14, which is known, and shaped in the shape which it is desired to impart to the transverse section of the extrusion 4 leaving the station: in practice, the billet 11, brought to the temperature of maximum plasticity specific to the alloy of which it is made, and once it has been introduced into the press 13 (which is preferably of the heated type), is subjected to an extremely high compression from a ram 15 of the press 13, which brings the alloy of which the billet 11 is composed into a fluid state, including if of high viscosity, which enables the alloy to flow through the die 14, receiving the desired shape from it and thus supplying, at the exit from the station 3, a solid pre-form (in the sense that it is capable of maintaining its own shape including under load and it can be handled mechanically), including if still red-hot, comprising the extrusion 4.

According to the method of the invention the extrusion phase, like every successive phase also, is carried out at the temperature of maximum plasticity of the alloy, and the extrusion 4 is formed as a tube which is substantially rectilinear and of substantially circular transverse section. More specifically, all the phases of the method of the invention are carried out whilst maintaining the alloy at a temperature at which it is in a semi-solid state, or it is within its solidification range and contains a liquid phase fraction lower than 50% by weight. According to a possible variant, however, at least the extrusion phase could also be carried out at a higher temperature, starting, for example, directly from the melt as well as from billets 11, in which case a different press 13 will be used and the die 14 will be of the cooled type, so as to ensure, however, at the exit from the station 3, the supply of an extrusion 4 which is at the temperature of maximum plasticity of the alloy used.

According to the invention the moulds 6, 7 of the station 5 are made of material that is a good conductor of heat and are provided with heating means, shown diagrammatically by 20 and capable of keeping them and, consequently, the blank 4 fed between them substantially at the same temperature at which it left the station 3, or at the above-mentioned temperature of maximum plasticity of the alloy used; the means 20 may be electrical resistors or, preferably, coils in which an oil (or another diathermic fluid heated in a suitable boiler which is not shown) is made to circulate.

Still according to the invention, furthermore, the moulding station 5 comprises actuating means 22 (comprising, for example, a hydraulic press with appropriate limit switches, shown solely in diagrammatic form with a block) capable of moving the moulds 6, 7 relatively in the direction of the arrow (Fig. 1) - generally speaking the mould 6 will be stationary and the mould 7 will be moved so that it is brought close to/moved away vertically from the mould 6 - to keep the moulds 6, 7 selectively arranged in two different operating positions.

A first operating position is that shown in Figs. 1 and 3, in which the moulds 6, 7 are arranged exactly superimposed, but only semi-close together, i.e. close together at a certain distance D apart from each other (Fig. 3) so that the facing cavities 8, 9 define between them an open guide channel 23 (in this case U-shaped on plan) for the extrusion 4; the cavities 8, 9 are also produced in such a way that the channel 23 is provided with at least one through open end 24 (see also Fig. 2) which is arranged in correspondence to the roller 10, facing towards the extrusion station 3, and through which the extrusion 4 leaving the station 3 can be introduced into the channel 23 to be caused to slide inside it, guided, for example, in contact with the bottom walls and/or the longitudinal corners of the semi-close together cavities 8, 9.

In contrast the second operating position which the moulds 6, 7 can assume is not shown, insofar as it corresponds simply to the first, but in which the distance D is reduced to zero, so that the moulds 6, 7 are kept close together with a pre-determined pressure; in particular, according to the invention the moulds 6, 7 are configured (or equipped, as will be seen) in such a way that in this second operating position they are close together not only in contact but also in a perfectly fluid-tight, particularly gas-tight, manner.

Finally the station 5 comprises pneumatic means, shown diagrammatically by 26, which are arranged, for example, incorporated inside (or underneath or adjacent to) the stationary mould 6, can be actuated solely in the second operating position of the moulds 6, 7 and are capable both of creating the vacuum inside the cavities 8, 9 between the extrusion 4, previously introduced into the channel 23, and the cavities 8, 9 themselves, and of conveying a pressurized gas inside the extrusion 4 which is present between the moulds 6, 7. In order to prevent possible corrosive phenomena of the extrusion 4, this gas is preferably an inert gas, such as helium, argon or nitrogen.

According to the method of the invention, once a substantially traditional extrusion phase has been carried out in the station 3, which produces an extrusion 4 of simple shape, so that the extrusion phase can be carried out at low cost, high speed and efficiency and with no waste, a phase of pre-forming or blocking towards the definitive shape desired for the box 2 is then carried out on the extrusion 4. For this purpose the block or blank which the tubular extrusion 4 constitutes is taken from the die 14 and immediately fed continuously, still hot, between the two moulds 6, 7 arranged in the above-mentioned first operating position, inside the curved channel 23 defined by the cavities 8, 9.

Thanks to the fact that the extrusion 4 is still at the temperature of maximum plasticity of the alloy which forms it (which is variable with the composition of the alloy and is therefore specific to each alloy used at any given time) and to the fact that it is maintained at this temperature by the means 20, the extrusion 4 is pre-formed by the effect of its sliding, with gradual introduction, in the channel 23 of which it will tend to assume the shape, in particular the extrusion 4 will be bent into a U (dashed section in Fig. 1) or into any other shape corresponding to the shape on plan of the cavities 8, 9.

When the introduction of the extrusion 4 into the channel 23 is completed, i.e. after the second phase, a third phase of the method of the invention is carried out which comprises a moulding phase of the already pre-formed extrusion into the definitive dimensions and shape of the box 2 to be obtained. Before this third phase is carried out, however, a cutting phase (Fig. 2) is carried out in which the pre-formed extrusion 4 in the channel 23 is cut in correspondence with the through open end 24 of the channel 23, by means of a bulkhead with shears 30, for example, which is made to ascend from a seat (not shown) provided in the mould 6 to intercept and close the end 23.

This same bulkhead 30 is produced in such a way that it is also capable of sealing the end 23 in a fluid-tight manner immediately after having carried out the cutting phase; alternatively, this closing function may be performed by any other known mobile sealing means, such as another sliding bulkhead, an expanding sleeve etc. In any event, immediately after the cutting phase (or also at the same time as it takes place) the moulds 6, 7 are brought together into contact, gradually reducing the distance D between them, until they are pressed against each other in a fluid-tight manner; in this configuration (Fig. 2) the bulkhead 30 (or means equivalent to it) will not only close the open end of the moulds 8, 9 in a fluid-tight manner but also the internal volume of the pre-formed extrusion 4, whose corresponding open end, or that just cut, will be coupled in contact with the bulkhead 30 (or with the possible sealing means which will have taken the place of the bulkhead/shears 30 after the cutting phase).

It is obvious that by bringing the moulds 6, 7 close together into contact, the cavities 8, 9 are also brought into contact, obtaining the deformation in the radial direction of the blank constituted by the extrusion 4, which is consequently subjected to the phase of moulding into the box 2 to be obtained. According to the invention, the moulding phase is not, therefore, carried out in traditional manner, simply by bringing the moulds 6, 7 into contact, but, profiting from the fact that the latter are brought close together in a fluid-tight manner and that, also once the moulds 6, 7 are close together the extrusion 4 is kept by the heating means 20 at the temperature of maximum plasticity of the alloy being worked, so that it is highly deformable, the moulding phase is carried out by creating a vacuum between extrusion 4 and cavities 8, 9, inside the cavities 8, 9 themselves, and by conveying a pressurized gas inside the extrusion 4.

For example, for this purpose the pneumatic means 26 include a double pump 40 and two pipes 41 and 42; the pipe 42 has an outlet (or a series of outlets, consequent on a possible bifurcation of it, which is not shown for reasons of simplicity) inside the cavities 8 and/or 9, whereas the pipe 41 extends partly inside the bulkhead 30, or in such a way as to have an outlet 44 facing, with moulds 6, 7 close together in contact, the internal cavity of the extrusion 4, in correspondence with one of its two opposite terminal ends, in the case illustrated one end 50 (Fig. 2) corresponding to the open end 24 (now closed by the bulkhead 30) of the channel 23. The opposite end (not illustrated for reasons of simplicity) of the extrusion 4 will now be sealed fluid-tight, either because it rests against closed and adjacent ends 52 (Fig. 1) of the cavities 8, 9 opposite the ends defining the open end 24, or because this end also of the extrusion 4 will be kept closed by a mobile bulkhead of the moulds 6, 7.

During the moulding phase according to the invention, therefore, the pressurized gas (inert gas such as argon, helium or nitrogen at 100 atmospheres, indicated by the small arrows in Fig. 3) fed inside the extrusion 4 through the channel 41 will tend to "inflate" it, producing the deformation of its lateral wall (the alloy forming the extrusion 4 is in fact in a plastic state) which is squeezed to copy the profile of the cavities 8, 9, whilst a similar effect will be achieved by the extraction of the air present in the cavities 8, 9 (only shown in diagrammatic form in Fig. 3 by small arrows pointing towards the pipe 42), which enables the plastic walls of the extrusion 4 in deformation phase to copy the walls of the cavities 8, 9 without air bubbles being interposed to produce surface defects.

Once a desired degree of vacuum has been reached inside the cavities 8, 9 and/or a desired pressure inside the blank 4, or a pre-determined time has elapsed, the heating means 20 are de-activated and the moulds 5, 6 moved apart to a distance greater than D and such as to enable the box 4 thus obtained to be extracted from them as soon as it has cooled down sufficiently.

By operating as described, starting from billets of aluminium alloy of the following composition by weight: 0.95% Si, 0.17% Fe, 0.5% Mn, 0.65% Mg, remainder Al, produced by Hydro Aluminium Sunndal (Norway), work is carried out in all the phases (extrusion, pre-forming and moulding) at the temperature of 575 °C, using an extrusion pressure of 1000 tonnes and carrying out the moulding at a gas pressure inside the blank of 100 atm and at industrial pressure on the outside, so as to eliminate the air space usually present between moulds and blank in a normal moulding phase. Tubular boxes of different shapes which are perfect and free from defects have been obtained in trials.

The technology of the invention can therefore be used for any light alloy and in particular for the alloys of aluminium (Al) such as: Al/copper, Al/silicon, Al/magnesium, Al/zinc alloys; and for magnesium (Mg)-based alloys such as: Mg/aluminium, Mg/aluminium/zinc, Mg/zinc/rare earths.

## Claims

1. Method for the hot-forming of a tubular box of any shape made from a light alloy, comprising a first phase in which the alloy is hot-extruded through a die (14) of suitable shape so as to be formed into a tube of pre-determined section and generally rectilinear, and a moulding phase, in which the extrusion (4) is moulded, to obtain the box of desired shape, between at least two moulds (6, 7) provided with respective conjugated cavities (8, 9) capable of defining with their contour the final shape of the box; **characterized in that** during the said moulding phase, the said moulds (6, 7) are kept close to each other in a fluid-tight manner; the said moulds being heated so as to maintain the extrusion (4), during the entire moulding phase, substantially at the same temperature at which it left the first extrusion phase; the moulding phase being carried out by creating a vacuum between extrusion (4) and cavities (8, 9), inside the cavities (8, 9), and conveying a pressurized gas inside the extrusion (4).

2. Method according to Claim 1 **characterized in that** it also comprises a second phase in which the extruded tube (4), still hot, is fed between the said moulds (6, 7) provided with conjugated cavities, during this second phase the moulds being heated so as to maintain the extrusion (4) substantially at the same temperature at which it left the first extrusion phase; during the second phase the moulds (6, 7) being kept close together at a certain distance apart from each other, so that the cavities (8, 9) define a guide channel (23) for the extrusion (4), inside which the latter is caused to slide so as obtain a pre-form of it.

3. Method according to Claim 2, **characterized in that** the said moulding phase is carried out after the said second phase, that of pre-forming, so as to constitute in sequence solely a third phase of the forming cycle of the box to be obtained; all the said phases being carried out with the alloy being kept in a temperature range around the temperature of maximum plasticity specific to the alloy used.

4. Method according to Claim 2 or 3, **characterized in that** the said second phase is carried out immediately downstream of the first phase, feeding the extrusion leaving the die (14) directly between the said semi-close together moulds (6, 7) and producing the latter in such a way that the said -guide channel (23) defined by said cavities (8, 9) of the moulds (6, 7) terminates towards the said die (14) with a through open end (24).

5. Method according to Claim 4, **characterized in that** after the second phase and before bringing the moulds (6, 7) close together in a fluid-tight manner to carry out the said moulding phase, the said extrusion (4) is cut in correspondence with the said through open end (24) of the guide channel (23) defined by the cavities (8, 9) of the moulds (6, 7); during the said moulding phase, the said open end (24) of the channel and the internal volume of the said extrusion (4) are closed in a fluid-tight manner by mobile sealing means (30).

6. Method according to one of the preceding Claims, **characterized in that** the said first phase, that of extrusion, is carried out starting from billets (11) cast in the light alloy of which it is desired to obtain the box, which billets are heated to the temperature of maximum plasticity of the alloy and then introduced into an extrusion press (13) one at a time.

7. Method according to Claim 6, **characterized in that** the said extrusion (4) is formed as a tube of substantially circular transverse section.

8. Method according to one of the preceding Claims, **characterized in that** all the said phases are carried out with the alloy being kept at a temperature at which it is in a semi-solid state, or it is within its solidification range and contains a liquid phase fraction less than 50% by weight.

9. Apparatus (1) for the hot-forming of a tubular box (2) of any shape made from a light alloy, comprising an extrusion station (3) capable of providing a tubular extrusion (4) of pre-determined section and generally rectilinear, and a moulding station (5) comprising at least two moulds (6, 7) provided with respective conjugated cavities (8, 9) capable of defining with their contour the final shape of the box to be obtained; **characterized in that** the said moulding station (5) is arranged immediately downstream of the extrusion station (3), to receive said extrusion (4) leaving the extrusion station (5) directly between said moulds (6, 7); the said moulds (6, 7) being provided with heating means (20) and the moulding station (5) also comprising:
- means (22) for keeping the moulds selectively arranged in two different operating positions, in a first of which the moulds (6, 7) are close together at a certain distance apart from each other, so that the cavities (8, 9) define a guide channel (23) for the extrusion (4) provided with a through open end (24) facing the extrusion station (3) and through which the extrusion (4) is capable of sliding in the channel (23) so as to be pre-formed by it; and in a second of which the said moulds (6, 7) are kept close together in a fluid-tight manner; and
- means (26) which can be actuated in the said second operating position of the moulds to create a vacuum between extrusion (4) and cavities (8, 9), inside the cavities, and to convey a pressurized gas inside the extrusion.

10. Apparatus according to Claim 9, **characterized in that** the said moulding station (5) also comprises mobile sealing means (30) capable, in said second operating position of the moulds (6, 7), of sealing in a fluid-tight manner the said through open end (24) of the channel (23) and the internal volume of the said extrusion (4).

## Patentansprüche

1. Verfahren zur Warmverformung eines aus einer Leichtmetalllegierung hergestellten röhrenförmigen Kastenprofils von beliebiger Form, umfassend eine erste Phase, in der die Legierung durch eine Düse (14) von geeigneter Form warmstranggepresst wird, so daß sie in ein Rohr mit vorbestimmtem Querschnitt und allgemein geradlinig geformt wird, und eine Formgebungsphase, in der das Strangpressprofil (4) zum Erhalten des Kastenprofils von gewünschter Form zwischen mindestens zwei Formen (6, 7) nachgeformt wird, die mit jeweiligen konjugierten Hohlräumen (8, 9) versehen sind, die mit ihrem Umriß die Endform des Kastenprofils definieren können; **dadurch gekennzeichnet**, daß während der besagten Formgebungsphase die besagten Formen (6, 7) auf eine fluiddichte Weise dicht zusammengehalten werden; wobei die Formen erwärmt werden, um das Strangpressprofil (4) während der ganzen Formgebungsphase im Wesentlichen auf derselben Temperatur zu halten, mit der es die erste Strangpressphase verließ; wobei die Formgebungsphase durchgeführt wird, indem ein Vakuum zwischen Strangpressprofil (4) und Hohlräumen (8, 9) innerhalb der Hohlräume (8, 9) erzeugt wird und ein Druckgas ins Innere des Strangpressprofils (4) gefördert wird.

2. Verfahren nach Anspruch 1, **dadurch gekennzeichnet**, daß es auch eine zweite Phase umfaßt, in der das stranggepresste Rohr (4) noch warm zwischen die mit konjugierten Hohlräumen versehenen besagten Formen (6, 7) zugeführt wird, wobei die Formen während dieser zweiten Phase erwärmt werden, so daß das Strangpressprofil (4) im Wesentlichen auf derselben Temperatur gehalten wird, mit der es die erste Strangpressphase verließ; wobei die Formen (6, 7) während der zweiten Phase in einem gewissen Abstand voneinander nahe beisammen gehalten werden, so daß die Hohlräume (8, 9) einen Führungskanal (23) für das Strangpressprofil (4) begrenzen, in dessen Innerem eine Verschiebung des Letzteren bewirkt wird, um einen Vorformling von ihm zu erhalten.

3. Verfahren nach Anspruch 2, **dadurch gekennzeichnet**, daß die Formgebungsphase nach der besagten zweiten Phase, der eines Vorformens, durchgerührt wird, so daß sie der Reihe nach nur eine dritte Phase des Formgebungszyklus des zu erhaltenden Kastenprofils bildet; wobei sämtliche besagten Phasen durchgeführt werden, wobei die Legierung in einem Temperaturbereich um die Temperatur einer maximalen Plastizität gehalten wird, die spezifisch für die verwendete Legierung ist.

4. Verfahren nach Anspruch 2 oder 3, **dadurch gekennzeichnet**, daß die zweite Phase in Bewegungsrichtung unmittelbar hinter der ersten Phase durchgeführt wird, wobei das die Düse (14) verlassende Strangpressprofil direkt zwischen die besagten halbnahe beisammen angeordneten Formen (6, 7) zugeführt wird und die Letzteren auf eine solche Weise hergestellt werden, daß der besagte Führungskanal (23), der durch die Hohlräume (8, 9) der Formen (6, 7) definiert ist, in Richtung auf die besagte Düse (14) mit einem offenen Durchgangsende (24) endet.

5. Verfahren nach Anspruch 4, **dadurch gekennzeichnet**, daß nach der zweiten Phase und bevor die Formen (6, 7) auf eine fluiddichte Weise dicht zusammengebracht werden, um die besagte Formgebungsphase durchzuführen, das besagte Strangpressprofil (4) in Übereinstimmung mit dem besagten offenen Durchgangsende (24) des Führungskanals (23), der durch die Hohlräume (8, 9) der Formen (6, 7) definiert ist, durchtrennt wird; und daß das besagte offene Ende (24) des Kanals und das Innenvolumen des besagten Strangpressprofils (4) während der besagten Formgebungsphase auf eine fluiddichte Weise durch bewegliche Dichteinrichtungen (30) verschlossen sind.

6. Verfahren nach einem der vorangehenden Ansprüche, **dadurch gekennzeichnet**, daß die erste Phase, diejenige des Strangpressens, ausgehend von Blöcken (11) durchgeführt wird, die aus der Leichtmetalllegierung gegossen werden, aus der man das Kastenprofil erhalten möchte, welche Blöcke auf die Temperatur einer maximalen Plastizität der Legierung erwärmt werden und dann einer nach dem anderen in eine Strangpresse (13) zugeführt werden.

7. Verfahren nach Anspruch 6, **dadurch gekennzeichnet**, daß das besagte Strangpressprofil (4) als Rohr von im Wesentlichen kreisförmigem Querschnitt geformt wird.

8. Verfahren nach einem der vorangehenden Ansprüche **dadurch gekennzeichnet**, daß sämtliche der besagten Phasen durchgeführt werden, wobei die Legierung auf einer Temperatur gehalten wird, bei der sie in einem halbfesten Zustand ist oder sich in ihrem Erstarrungsbereich befindet und einen Flüssigphasenanteil von weniger als 50 Gew.-% enthält.

9. Vorrichtung (1) zur Warmverformung eines aus einer Leichtmetalllegierung hergestellten röhrenförmigen Kastenprofils (2) von beliebiger Form, umfassend eine Strangpressstation (3), die ein röhrenförmiges Strangpressprofil (4) mit vorbestimmtem Querschnitt und allgemein geradlinig bereitstellen kann, und eine Formgebungsstation (5), die mindestens zwei Formen (6, 7) umfaßt, welche mit jeweiligen konjugierten Hohlräumen (8, 9) versehen sind, die mit ihrem Umriß die Endform des zu erhaltenden Kastenprofils definieren können; **dadurch gekennzeichnet**, daß die Formgebungsstation (5) in Bewegungsrichtung unmittelbar hinter der Strangpressstation (3) angeordnet ist, um das die Strangpressstation (5) verlassende Strangpressprofil (4) direkt zwischen den Formen (6, 7) aufzunehmen; wobei die Formen (6, 7) mit Heizeinrichtungen (20) versehen sind und die Formgebungsstation (5) auch umfaßt:
- Einrichtungen (22), um die Formen wahlweise in zwei unterschiedlichen Betriebsstellungen zu halten, in deren erster die Formen (6, 7) in einem gewissen Abstand voneinander nahe beisammen sind, so daß die Hohlräume (8, 9) einen Führungskanal (23) für das Strangpressprofil (4) definieren, der mit einem offenen Durchgangsende (24) versehen ist, das der Strangpressstation (3) gegenüberliegt und durch das sich das Strangpressprofil (4) in den Kanal (23) schieben kann, so daß es durch ihn vorgeformt wird; und in deren zweiter die besagten Formen (6, 7) auf eine fluiddichte Weise dicht zusammengehalten werden; und
- Einrichtungen (26), die in der zweiten Betriebsstellung der Formen betätigt werden können, um ein Vakuum zwischen Strangpressprofil (4) und Hohlräumen (8, 9) innerhalb der Hohlräume zu erzeugen und um ein Druckgas ins Innere des Strangpressprofils zu fördern.

10. Vorrichtung nach Anspruch 9, **dadurch gekennzeichnet**, daß die Formgebungsstation (5) auch bewegbare Dichtungseinrichtungen (30) umfaßt, die in der zweiten Betriebsstellung der Formen (6, 7) das besagte offene Durchgangsende (24) des Kanals (23) und das Innenvolumen des besagten Strangpressprofils (4) auf eine fluiddichte Weise abdichten können.

## Revendications

1. Procédé pour le formage à chaud d'un caisson tubulaire de forme quelconque en alliage léger, comprenant une première phase dans laquelle l'alliage est extrudé à chaud à travers une filière (14) de forme appropriée afin de produire un tube de section prédéterminée et sensiblement rectiligne, et une phase de moulage dans laquelle l'extrusion (4) est moulée de manière à obtenir le caisson de forme désirée, entre au moins deux moules (6, 7) comportant des cavités conjuguées respectives (8, 9) dont le contour peut définir la forme finale du caisson ; **caractérisé en ce que**, pendant la dite phase de moulage, les dits moules (6, 7) sont maintenus l'un près de l'autre d'une manière étanche aux fluides ; les dits moules sont chauffés de façon à maintenir l'extrusion (4), pendant toute la phase de moulage, sensiblement à la même température à laquelle elle a quitté la première phase d'extrusion, la phase de moulage étant effectuée par création d'un vide entre l'extrusion 4 et les cavités (8, 9), à l'intérieur des cavités (8, 9), et par amenée d'un gaz sous pression à l'intérieur de l'extrusion (4).

2. Procédé selon la revendication 1, **caractérisé en ce qu**'il comprend également une deuxième phase dans laquelle le tube extrudé (4), encore chaud, est amené entre les dits moules (6, 7) comportant des cavités conjuguées, les moules étant chauffés pendant cette deuxième phase de manière à maintenir l'extrusion (4) sensiblement à la même température à laquelle elle a quitté la première phase d'extrusion, les moules (6, 7) étant maintenus l'un près de l'autre et à une certaine distance l'un de l'autre pendant la deuxième phase, de sorte que les cavités (8, 9) définissent un canal de guidage (23) de l'extrusion (4), à l'intérieur duquel cette denière peut glisser afin de produire une ébauche de l'extrusion.

3. Procédé selon la revendication 2, **caractérisé en ce que** la dite phase de moulage est effectuée après la dite deuxième phase, celle du préformage, de façon à constituer en séquence seulement une troisième phase du cycle de formage du caisson à obtenir, toutes les dites phases étant effectuées tandis que l'alliage est maintenu dans une plage de température autour de la température de plasticité maximale spécifique de l'alliage utilisé.

4. Procédé selon la revendication 2 ou 3, **caractérisé en ce que** la dite deuxième phase est effectuée immédiatement en aval de la première phase, on amène l'extrusion sortant de la filière (14) directement entre les dits moules à demi-fermés (6, 7) et on prépare ces derniers d'une manière telle que le dit canal de guidage (23) défini par les dites cavités (8, 9) des moules (6, 7) se termine vers la dite filière (14) par une extrémité ouverte traversante (24).

5. Procédé selon la revendication 4, **caractérisé en ce que**, après la deuxième phase et avant d'amener les moules (6, 7) en position fermée d'une manière étanche aux fluides afin d'exécuter la dite phase de moulage, on coupe la dite extrusion (4) en correspondance de la dite extrémité ouverte traversante (24) du canal de guidage (23) défini par les cavités (8, 9) des moules (6, 7) et, pendant la dite phase de moulage, la dite extrémité ouverte (24) du canal et le volume intérieur de la dite extrusion (4) sont fermés d'une manière étanche aux fluides par des moyens d'obturation mobiles (30)/

6. Procédé selon une des revendications précédentes, **caractérisé en ce que** la dite première phase, celle d'extrusion, est effectuée en partant de billettes (11) coulées en l'alliage léger avec lequel on désire fabriquer le caisson, ces billettes étant chauffées à la température de plasticité maximale de l'alliage puis introduites une par une dans une presse d'extrusion (13).

7. Procédé selon la revendication 6, **caractérisé en ce que** la dite extrusion (4) est sous la forme d'un tube de section transversale sensiblement circulaire.

8. Procédé selon une des revendications précédentes, **caractérisé en ce que** toutes les dites phases sont exécutées tandis que l'alliage est maintenu à une température à laquelle il est dans un état semi-solide, ou bien il est dans sa plage de solidification et contient une fraction de phase liquide inférieure à 50% en poids.

9. Appareil (1) pour le formage à chaud d'un caisson tubulaire (2) de forme quelconque en un alliage léger, comprenant une station d'extrusion (3) pouvant fournir une extrusion tubulaire (4) de section prédéterminée et sensiblement rectiligne, et une station de moulage (5) incluant au moins deux moules (6, 7) qui présentent des cavités conjuguées respectives (8, 9) dont le contour peut définir la forme finale du caisson à obtenir, **caractérisé en ce que** la dite station de moulage (5) est placée immédiatement en aval de la station d'extrusion (3) pour recevoir la dite extrusion (4) sortant de la station d'extrusion (5) directement entre les dits moules (6, 7), les dits moules (6, 7) étant pourvus de moyens de chauffage (20) et la station de moulage (5) comprenant également :
des moyens (22) de maintien des moules sélectivement agencés dans deux positions de fonctionnement différentes, dans une première desquelles les moules (6, 7) sont rapprochés à une certaine distance l'un de l'autre de sorte que les cavités (8, 9) définissent un canal de guidage (23) pour l'extrusion (4) ayant une extrémité ouverte traversante (24) en regard de la station d'extrusion (3) et à travers laquelle l'extrusion (4) peut glisser dans le canal (23) de façon à être préformée par celui-ci, et dans une deuxième desquelles les dits moules (6, 7) sont maintenus fermés l'un contre l'autre d'une manière étanche aux fluides, et
des moyens (26) qui peuvent être actionnés, dans la dite deuxième position de fonctionnement des moules, pour créer un vide entre l'extrusion (4) et les cavités (8, 9), à l'intérieur des cavités, et pour amener un gaz sous pression à l'intérieur de l'extrusion.

10. Appareil selon la revendication 9, **caractérisé en ce que** la dite station de moulage (5) comprend également des moyens d'obturation mobiles (30) qui peuvent, dans la dite deuxième position de fonctionnement des moules (6, 7), fermer de façon étanche aux fluides la dite extrémité ouverte traversante (24) du canal (23) et le volume intérieur de la dite extrusion (4).
